

# UNITED STATES PATENT OFFICE.

ROBERT D. PIKE, OF RICHMOND, CALIFORNIA.

## CARBON AND METHOD OF MANUFACTURING SAME.

1,262,251.

Specification of Letters Patent.

Patented Apr. 9, 1918.

No Drawing.

Application filed December 21, 1915. Serial No. 63,088.

To all whom it may concern:

Be it known that I, ROBERT D. PIKE, a citizen of the United States, residing at Richmond, in the county of Contra Costa 5 and State of California, have invented certain new and useful Improvements in Carbons and Methods of Manufacturing Same, of which the following is a specification.

The present invention relates to electric 10 light carbons, mainly designed for use as "projector" carbons, and the invention resides in the production of carbons for use generally from what is commonly known as "lamp black" refuse derived from the 15 manufacture of illuminating gas from crude petroleum.

I have discovered that carbons produced from the so-called "lamp black" refuse from the manufacture of illuminating gas from 20 crude petroleum possess certain qualities lacking in the ordinary carbons, noticeably the ability of the carbons to be carried very close together while burning and even to be frozen, without hissing. This is a feature 25 which no other carbon possesses, and its advantage is two fold. First, carbons give a greater luminous efficiency when carried close with a short arc, and secondly, it is much easier for the operator to adjust the 30 carbons when displaying a picture if he is not called on to be continuously guarding against hissing. Again, the carbons produced from the so-called "lamp black" refuse of the gas plant have a higher current carrying 35 capacity than the carbons as ordinarily made and employed for use in projecting machines, as, for example, I can employ a  $\frac{3}{8}$ " carbon to carry from sixty to seventy amperes, while with the ordinary carbon a 40  $\frac{3}{8}$ " carbon is required for the carrying of a similar current.

I have found that the so-called "lamp black" refuse from the manufacture of illuminating gas from crude petroleum, per hundred pounds contains the following in about 45 the proportions given:—

Three pounds of soluble and insoluble ash, of which two and one half pounds is soluble; tar, thirty pounds; hydrocarbons, soluble at 50 low temperature, ten pounds; water, thirty pounds; lamp black, twenty-seven pounds.

In carrying out my process for the manufacture of the carbons from the mentioned lamp black, the first of the impurities to be 55 eliminated is the tar.

For this purpose the mass of refuse matter

is subjected to hot water washing and milling in what is known as a "chaser" mill or wet pan. This operation, which is carried on for a period of approximately twenty 60 minutes agglomerates the tar into pellets about the size of a pea and flat wafers, which are separated by washing in a screen of suitable mesh. The resultant product is finely divided lamp black, which is treated 65 for the elimination of soluble ash by any suitable washing apparatus, wherein the washing is done with successive charges of water, each charge being drained off for washing away the soluble ash. The material with the soluble ash eliminated therefrom is 70 treated in a roaster or drier, wherein it is agitated while subjected to a temperature of approximately 1000 degrees Fahr., for the removal of all moisture and the high volatile 75 hydrocarbons. This roasting is continued for approximately three hours, after which the material is in a dry powdered form, but still contains a trace of hydrocarbon volatiles and from five to ten per cent. by weight 80 of occluded air. To eliminate these features, the material is then charged in fire clay muffles and subjected to a bright red heat at a temperature of between 1800 degrees to 2000 degrees Fahr., and subjected to 85 such roasting for eighteen hours.

The resultant product is lamp black, containing approximately one per cent. of volatile matter and one and one-half per cent. of insoluble ash.

After the material has become cool it is 90 ground in a suitable mill and reduced to a fine powder, which is run through separators to remove iron particles which may be contained therein. A suitable flux is then added 95 for the small per cent. of insoluble ash remaining therein, and thereafter, by the intermixing therewith of a small quantity of coal tar, the mixture is run through suitable rolls to produce a plastic body, which is 100 then compressed into cylindrical cakes. These cakes are formed into green carbon sticks, which are baked in the usual manner for forming carbons.

The carbons produced from the so-called 105 lamp black refuse of the plants manufacturing illuminating gas from crude oil have proved to be more efficient than the carbons at present in use, with reference more particularly for use in connection with projecting apparatus.

Having thus described the invention what

is claimed as new and desired to be protected by Letters Patent is:—

1. The method of purifying the lamp black refuse derived from the manufacture of illuminating gas from crude oil, which consists first in eliminating therefrom by washing the tar contained therein, then by washing removing the soluble ash, then roasting under agitation for the removal of moisture and the high volatile hydrocarbons, and then roasting at a higher temperature for the elimination of remaining hydrocarbons.
2. The method of purifying the lamp black

refuse derived from the manufacture of illuminating gas from crude oil, which consists first in eliminating from the material by washing and roasting the impurities contained therein, and then reducing the material to a powder form. 15

In testimony whereof I have signed my name of this specification in the presence of two subscribing witnesses. 20

ROBERT D. PIKE.

Witnesses:

C. F. LINDSEY,  
W. H. CONN.